

## UNITED STATES PATENT OFFICE.

DANIEL D. JACKSON, OF BROOKLYN, NEW YORK; JOSEPH D. SEARS, OF BLOOMFIELD, AND FREDERICK CONLIN, OF WESTFIELD, NEW JERSEY, ASSIGNEES TO JOHN T. PRATT, OF NEW YORK, N. Y.; DANIEL D. JACKSON, OF BROOKLYN, NEW YORK, AND JOSEPH D. SEARS, OF BLOOMFIELD, NEW JERSEY, TRUSTEES.

PROCESS OF DESULPHURIZING IRON, STEEL, FERRO ALLOY, AND COMPOSITIONS OF MATTER FOR USE THEREIN.

No Drawing.

Application filed July 29, 1922. Serial No. 578,485.

To all whom it may concern:

Be it known that we, DANIEL D. JACKSON, residing in the borough of Brooklyn, city and State of New York, JOSEPH D. SEARS, residing in Bloomfield, county of Essex, and State of New Jersey, and FREDERICK CONLIN, residing in Westfield, county of Union, and State of New Jersey, citizens of the United States of America, have invented certain new and useful Improvements in Processes of Desulphurizing Iron, Steel, Ferro Alloys, and Compositions of Matter for Use Therein, of which the following is a specification.

This invention relates to a process of desulphurizing iron, steel, and ferro-alloys, and to compositions of matter for use in such process, and aims to provide improvements therein.

We have discovered that alkaline reagents, such as caustic soda, sodium carbonate, and mixtures thereof, used for desulphurizing, have an effect in removing silicon from iron, steel, etc., in addition to sulphur, and this removal of silicon is undesirable in certain cases, as where the iron, steel, etc. is to be used for casting, particularly in the manufacture of gray iron castings.

The present invention provides a process whereby iron, steel, etc. may be desulphurized by the use of alkaline reagents, and notably caustic soda, sodium carbonate, or mixtures thereof, without reduction in silicon.

The invention further provides a composition of matter for use in said process, for desulphurizing without reducing the silicon, as above set forth.

According to the present invention, caustic soda, sodium carbonate, or other alkaline reagent used for desulphurizing, and preferably a mixture of sodium carbonate and caustic soda in about the proportions of 70% sodium carbonate to 30% caustic soda (as set forth in our companion application Serial No. 631,925 filed April 18, 1923) and a silicon-alloy are added to the metal to be desulphurized.

The mixture of alkaline reagent and silicon-alloy is conveniently brought into contact with the metal in a ladle, the mixture

being introduced before, during or after the running in of the molten metal.

The silicon-alloy should preferably have a melting point below the temperature of the molten metal, in order that it may be melted by the heat of the metal. A ferro-silicon containing 60% silicon, having a melting point of about 2200° F., in admixture with the alkaline reagent, has given satisfactory results with iron and steel for casting.

The amount of the silicon-alloy to use will vary with the desiliconizing action of the alkaline reagent employed. As the alkaline reagent has a tendency to take out more silicon from the metal, more of the silicon-alloy will be required to counteract or replace the silicon removed or which would otherwise be removed, by the alkaline desulphurizing agent.

Satisfactory results in practice have been obtained when 5-20% by weight of the compound of the mixture of a ferro-silicon alloy containing 50 to 60% silicon has been incorporated with the desulphurizing combination of about 70% sodium carbonate and 30% caustic soda.

The amount of silicon-alloy to use in the case of different alloys and of different alkaline desulphurizing reagents is best found by experiment based on a knowledge of the desiliconizing action of the alkaline reagent.

The silicon-alloy ordinarily takes a longer time to melt than the alkaline reagent or mixture. By introducing the silicon-alloy in admixture, or concurrently, into the receptacle of the metal with the alkaline reagent, the silicon-alloy undergoes heating along with the alkaline reagent, and consequently reaches its melting point after the alkaline reagent has to a large extent completed its work. This in practice allows the alkaline reagent and silicon alloy to be melted by the heat of the metal in a ladle or receptacle, after having been run from a melting furnace, and before the metal in the ladle cools to a point which would interfere with the proper pouring of the metal from the ladle into molds. The delayed action of the silicon-alloy in melting is also of

advantage in that the desulphurizing compound may exert its full action on the molten metal without wasting part of its effect by a side reaction on the silicon in the silicon 5 alloy.

In treating iron for casting with ferro-silicon containing 60% silicon, it is found that it requires about 3 to 6 minutes for the ferro-silicon to melt, and this period is sometimes about as long as metal can stand in a ladle before becoming too chilled for pouring. The silicon-alloy is, however, found to have an exothermic reaction with the metal, so that its use counteracts the drop in temperature of the metal due to the use of the alkaline reagent, and enables the entire reaction to occur in the period in which the metal can ordinarily stand in a ladle before becoming too chilled for proper pouring. 15 The alkaline reagent and the silicon alloy are preferably mixed, the lower melting point constituents fused, and formed into lumps or flakes or cakes of convenient size. These lumps, flakes or cakes are only slightly 20 deliquescent, safe for handling, and have the characteristics in use above set forth. A size somewhat above powder particles, and larger, is found to very much facilitate the melting of the composition. 25 Other proportions than those specifically mentioned, and other procedures than those specifically given, may be adopted without departing from the idea of the invention. Moreover, it is understood that the invention 30 may be generally applied to the desulphurizing of metals.

What is claimed is:

1. A process of desulphurizing comprising treating molten iron, steel, and ferro-alloys with an alkaline desulphurizing reagent having a desiliconizing effect and a silicon-alloy.
2. A process of desulphurizing comprising treating molten iron, steel, and ferro-alloys with an alkaline desulphurizing reagent having a desiliconizing effect and a silicon-alloy having a melting point not substantially above the melting point of the metal.
3. A process of desulphurizing comprising treating molten iron, steel, and ferro-alloys with caustic soda and a silicon-alloy.

4. A process of desulphurizing comprising treating molten iron, steel, and ferro-alloys with sodium carbonate and a silicon-alloy. 55

5. A process of desulphurizing comprising treating molten iron, steel, and ferro-alloys with sodium carbonate and caustic soda and a silicon-alloy. 60

6. A process of desulphurizing comprising treating molten iron, steel, and ferro-alloys with an alkaline desulphurizing reagent having a desiliconizing effect and ferro-silicon containing in the neighborhood of 50-60% silicon. 65

7. A process of desulphurizing comprising treating molten iron, steel, and ferro-alloys with sodium carbonate and caustic soda substantially in the proportion of 70% sodium carbonate and 30% caustic soda, and ferro-silicon containing in the neighborhood of 50-60% silicon, the amount of said ferro silicon being 5-20% of the other ingredients. 70

8. A process of desulphurizing comprising running molten iron, steel, and ferro-alloys into a ladle or the like, and treating the metal with an alkaline desulphurizing reagent having a desiliconizing effect and a silicon-alloy having a melting point not substantially above the melting point of the metal, allowing the mixture to act for a short period, and pouring the metal while it is still fluid enough for running into molds. 75

9. A composition of matter comprising an alkaline desulphurizing reagent having a desiliconizing effect and a silicon-alloy. 85

10. A composition of matter comprising caustic soda and a silicon-alloy.

11. A composition of matter comprising sodium carbonate and a silicon-alloy. 90

12. A composition of matter comprising caustic soda, sodium carbonate and a silicon-alloy.

13. A composition of matter comprising caustic soda and sodium carbonate substantially in the proportions of 30% and 70% respectively, in which is incorporated ferro-silicon containing about 50-60% silicon. 95

In witness whereof, we have hereunto signed our names.

DANIEL D. JACKSON.  
JOSEPH D. SEARS.  
FREDK. CONLIN.